

## UNITED STATES PATENT OFFICE

2,121,799

## PROCESS FOR MAKING CAST PERMANENT MAGNETS

Hugh A. Howell, Berwyn, Ill., assignor to Frank Raffles, Chicago, Ill.

No Drawing. Application June 29, 1937.  
Serial No. 151,029

8 Claims. (Cl. 75—27)

This invention relates to cast permanent magnets and more particularly to a new process for their fabrication.

It is one of the objects of the present invention to provide a method of making cast magnets easily and cheaply without recourse to orthodox foundry methods, materials and equipment.

This invention relates particularly to the various new magnet alloys containing iron, nickel, aluminum and other ingredients in vary percentages.

One of the important objects of this invention is the provision of a simple, economical method of producing cast alloys which can be later readily magnetized and which, on account of the method of manufacture, will acquire and possess a high degree of magnetic power.

A further object of the invention is the provision of a magnetic alloy which eliminates the necessity of annealing or aging so far as the final product is concerned, particularly in that the super-heating, which accompanies the process of manufacture, produces a product which, when cooled, is practically automatically normalized.

My new process permits the making of cast magnets cheaply and quickly, either in the shop or laboratory, without the use of a furnace or the conventional molding equipment necessary in a foundry where small castings are made.

The new features which I believe to be characteristic of my invention are set forth in the following specifications and particularly in the appended claims.

My invention will be best understood from reference to the well-known chemical reaction between iron oxide and aluminum based on the equation  $Fe_2O_3 + 2Al = 2Fe + Al_2O_3$ . Iron oxide and metallic aluminum in a properly divided state, mixed in about the proportions of the foregoing equation, will react when properly ignited in such a way that the oxygen in the iron oxide is released and combines with the metallic aluminum to form aluminum oxide or slag, setting free the iron. The combustion is started by igniting the mixture at one spot and continues throughout the entire mass without the use of any other heating agency and results in super-heated liquid iron and slag. The complete reaction is completed in less than one half minute, creating a temperature in the neighborhood of 5000° F. The liquid iron produced represents one half of the original mixture by weight and one third by volume. The foregoing chemical reaction was first observed in 1857 by Friederich Woehler, the discoverer of aluminum.

In fabricating magnet alloys with my new process, I mix iron oxide in the proper physical state with aluminum, nickel or other metals in a divided and commercially pure state in an ordinary graphite crucible. I ignite this mixture with a small electric arc produced in any convenient manner. While the chemical reaction is taking place, I agitate the mixture by rocking and twirling the crucible, while holding in an upright position in order to cause the super-heated slag to freeze or adhere to the sides of the crucible. After the reaction has been completed, and before the liquid iron has had time to solidify, I pour all but the slag into an unheated carbon mold built up of several parts. Immediately after the casting has solidified, I remove it from the mold to cool naturally in the open air.

The cast material may be magnetized in a suitable manner either in one piece or after having been cut or broken into separate parts. Further machining, shaping and finishing may also be accomplished either before or after magnetizing.

I make my molds of pre-fabricated carbon sections, the number of sections depending upon the size and shape of the magnet and the amount of detail desired.

Cores and even parts of the mold can also be made of a mixture consisting of graphite one part and fine molding sand, two parts, with any good core binder. I fire all core and mold parts to remove water and carbonize the binder. I have made as high as one hundred castings from an all carbon mold. With a machined carbon mold properly designed, castings can be made that compare favorably with die castings in definition and accuracy. I find a carbon mold built up in parts particularly desirable in making very small and delicate castings.

In making a magnet alloy of the recently developed nickel, iron and aluminum variety, I use the following mixture in my process:

|                                                    | Parts by weight |
|----------------------------------------------------|-----------------|
| Iron oxide (scale)—approximately                   | 40              |
| Fine commercially pure aluminum shot—approximately | 15              |
| Fine nickel shot—approximately                     | 10              |

With above mixture and variations of same, I have poured castings weighing as little as five grams, the only equipment necessary being a pair of tongs, a small crucible and a suitable igniting device.

With a mixture consisting of 40 grams of iron oxide, 15 grams of aluminum shot and 10 grams

of nickel shot, a casting weighing about 35 grams may be produced.

The uniformity of magnet alloys made with my process is limited only by the accuracy in weighing out the mixture. It is a well-known fact that the presence of other metals and carbon in reasonably small percentages does not damage the magnetic properties of the nickel-aluminum-iron family of alloys. In fact, others have claimed 10 that the addition of a certain amount of cobalt, chromium, copper, vanadium or manganese, etc. gives improved characteristics to the alloys.

I have not observed any marked improvement by special heat treatment of magnets made by my 15 method, therefore heat treatment does not form a part of my process.

The mixture described, consisting of about 40 grams of flake iron oxide, 15 grams of shotted aluminum and 10 grams of nickel will, after the 20 chemical reaction is completed, produce about 35 grams of magnet alloy with approximately the following analysis and characteristics:

| 25 | Chemical composition |        |          | Magnetic properties         |                                 |
|----|----------------------|--------|----------|-----------------------------|---------------------------------|
|    | (Percent)            |        |          | Coercive force (HC) (Gauss) | Residual magnetism (BR) (Gauss) |
|    | Iron                 | Nickel | Aluminum |                             |                                 |
| 30 | 62                   | 28     | 10       | 250                         | 9,500                           |

It will be noted that when the crucible is whirled, the liquid slag, which will not mix with the metal and evidently has a higher melting point, freezes or solidifies in a thin strata on the sides of the still relatively cool crucible so that when the thermic action is completed, the liquid metal is easily poured out of the crucible, there being absolutely no slag in the pour. After the crucible has cooled to about 400° F. or lower, the layer of slag clinging to the sides and bottom of the crucible will drop out by simply inverting the crucible. It may sometimes be necessary to tap the bottom of the crucible with a wooden mallet. 45 In all cases, the slag formation drops out in a one-piece cup shape.

It will also be observed that the cooled magnet alloy will, under practically all conditions, retain 50 a silvery white untarnished finish, especially if carbon molds are used. The accuracy of castings seems to be limited only by the design and tolerances in the mold.

Alloys, when made with this process and poured 55 soon enough after the chemical reaction is completed, will be superheated and very liquid, as compared with ordinary foundry practice. I have filled in cavities in carbon molds resulting in fins over one inch square and less than .010 inch thick—proving the fluidity of alloy.

I am aware that many changes may be made 60 in the ingredients and numerous details in the process varied throughout a wide range without departing from the principles of this invention, and I, therefore, do not purpose limiting the patent granted hereon otherwise than as necessitated by the prior art.

What I claim as new in the fabrication of per-

manent magnet alloys and desire to secure by Letters Patent of the United States is:

1. The method of making a permanent magnet alloy consisting substantially of mixing by weight 30 to 50 parts iron oxide, 10 to 20 parts aluminum and 5 to 15 parts of nickel, and igniting in a crucible, rotating the crucible to freeze slag to the sides of the crucible, and pouring liquid metal into a mold after chemical action has been completed. 5

2. The method of making a permanent magnet 10 alloy consisting of mixing by weight 25 to 60 parts of flake iron oxide, 5 to 25 parts of shotted aluminum, and 2 to 20 parts of shotted nickel, igniting said mixture in a crucible, whirling the crucible to cause slag to solidify on sides of crucible, and pouring resultant liquid metal into a carbon mold immediately after chemical action 15 is completed.

3. The method of making a permanent magnet 20 alloy consisting substantially of mixing by weight 30 to 50 parts of flake iron oxide, 10 to 20 parts of fine shotted aluminum and 5 to 15 parts of fine shotted nickel; pouring this mixture in a graphite crucible and igniting said mixture; agitating with a whirling motion during chemical 25 reaction to freeze liquid slag to sides of crucible and pouring resultant liquid metal into a carbon mold after combustion is completed, removing the solidified casting and allowed to cool in air.

4. The method of making a permanent magnet 30 alloy consisting substantially of 30 to 50 parts of iron oxide and 10-20 parts nickel and 10-20 parts aluminum by weight, adding any other metals in the pure and properly divided state to produce the desired alloy, igniting in a crucible 35 and pouring into suitable molds after chemical action has been completed and slag has solidified on the sides of the crucible.

5. A method of making a permanent magnet, 40 which method comprises mixing iron oxide, aluminum and nickel in a crucible, igniting the mixture, separating out the slag, pouring the molten metal into a mold after the slag has solidified on the sides of the crucible, and then magnetizing the casting. 45

6. A method of making a magnetic alloy, comprising mixing flake iron oxide, aluminum and nickel in a crucible, igniting the mixture, centrifuging out the slag while the thermic reaction 50 is taking place and pouring the molten metal into molds. 50

7. A method of making a magnetic alloy, comprising mixing iron oxide, aluminum and nickel in a crucible in such proportions as to yield a final composition containing approximately iron 55 60%, nickel 30%, and aluminum 10%, igniting the mixture, separating the liquid from the slag by centrifugal action and pouring the molten metal into molds.

8. A method of making a magnetic alloy, comprising mixing iron oxide, aluminum and nickel in a crucible in such proportions as to yield a final composition containing approximately iron 60 50 to 70%, nickel 20 to 40%, and aluminum 8 to 15%, igniting the mixture, centrifuging out the 65 slag and pouring the molten metal into molds.

HUGH A. HOWELL.